

## UNITED STATES PATENT OFFICE

2,254,337

## HALOGENATED LUBRICANT

William A. Whittier, Kenilworth, Ill., assignor to  
The Pure Oil Company, Chicago, Ill., a corpora-  
tion of Ohio

No Drawing. Application September 23, 1938,  
Serial No. 231,342

26 Claims. (Cl. 252—48)

This invention relates to lubricants and is more particularly concerned with lubricants having high extreme pressure characteristics.

It is well known that the load carrying ability of mineral lubricating oils can be improved by adding thereto various halogenated hydrocarbons. It is also well known that a somewhat similar improvement in the load carrying ability of mineral lubricating oils can be effected by adding thereto lead soaps, sulfurized hydrocarbons, sulfurized fatty oils and phosphorus compounds.

The extent of the improvement accomplished by the various extreme pressure additives varies considerably depending upon a number of factors, some of the more important of which are the particular extreme pressure agent used, the quantity added and the testing method used to measure the load carrying capacity. Of these variables, perhaps the most difficult to correlate is the load carrying ability as indicated by different testing apparatus. There are a number of devices commercially available for determining the extreme pressure characteristics of lubricants, such as the Floyd, Almen, Faville-Levalley, Timken, S. A. E. and a number of others which test E. P. lubricants for more specific applications. Two of these machines appear to be much more widely accepted than any of the others. These are "The Timken Wear and Lubricant Tester" made by the Timken Roller Bearing Company of Canton, Ohio, and a machine offered as a tentative standard by the Society of Automotive Engineers and known as the "S. A. E. Extreme Pressure Testing Machine." This machine is made by the Highway Trailer Company of Edgerton, Wisconsin. Unfortunately there is considerable difference in the results obtained in the two machines and in the application of the results to practical lubricating problems. For example, mineral oil, to which has been added lead soap and active sulfur, will withstand the full load on the S. A. E. machine, 550 lbs. at 1000 R. P. M., whereas on the Timken machine the results are quite low, being of the order of 18 to 25 lbs. beam arm load and a pressure of 10,000-13,000 lbs. per square inch.

Lubricating engineers are not entirely in agreement as to just what these tests mean in actual performance, although there has been a great deal of work done to correlate such test results with actual service. At the present time it appears that the only entirely satisfactory test for E. P. lubricants is actual service, though the Timken and S. A. E. machines serve a useful purpose by indicating those lubricants that are worthy of the time and expense required for actual service tests. It is significant to note that commercially successful E. P. lubricants on the market at the present time give good results on

one or the other of these machines. It is equally significant that commercially successful E. P. lubricants will not withstand high loads on both the S. A. E. and Timken machines, that is, a load of the order of 300 lbs. at 1000 R. P. M. on the S. A. E. machine and 68 lbs. beam arm load and 25,000 lbs. per square inch on the Timken machine.

It is an object of this invention to provide an improved E. P. lubricant.

Another object of this invention is to provide an E. P. lubricant which will give superior results in actual service and will give satisfactorily high results on both the Timken and S. A. E. extreme pressure testing machines.

A further object of this invention is to provide a stable non-corrosive E. P. base and lubricant which when added to mineral lubricating oils will be entirely soluble and will impart unusual E. P. characteristics to the resulting blend without attacking the metal parts with which it comes in contact.

Still further objects of this invention will be apparent from the following description.

I have discovered that certain chlorinated open chain aliphatic hydrocarbons, when added to phosphorized or sulfurized and phosphorized lubricants of the non-corrosive type, for example such as those disclosed in application Serial No. 55,200, Whittier et al. and Chittick Patent No. 2,142,998, issued January 10, 1939, produce lubricants which do not hydrolyze, are completely soluble in mineral oil and show unexpectedly high results on both the Timken and S. A. E. testing machines. Service tests also show this lubricant to be far superior to any E. P. lubricant commercially available.

The sulfurized-phosphorized lubricant may be prepared in the following manner:

A homogeneous mixture of 570 pounds of Gulf Coast pale oil having a Saybolt Universal viscosity of 200 seconds and a pour point of -20° to -25° F. and 55 pounds of sulfur chloride is prepared in a cold state. This mixture is added to 9,581 pounds of prime lard oil contained in an enclosed steam jacketed kettle. The mixture is heated to 275° F. while being vigorously agitated. At this point the steam is shut off and 814 pounds of flowers of sulfur are sifted into the contents of the kettle over a period of approximately two hours. The contents of the kettle are vigorously agitated during this entire period. At the end of a two-hour period the temperature will have dropped to 265° F. The steam is again turned on and the contents of the kettle heated to approximately 300° F. at which time the steam is turned off. Agitation is continued for a period of approximately 7½ hours after the addition of the sulfur. During this period the temperature will have risen from 300° to 344° F. during the first

three hours indicating that an exothermic reaction was taking place. The temperature during the 7½-hour period is not permitted to drop below 320° to 330° F. and it has been found that it is unnecessary to use any further heat to maintain this temperature after the mixture has been initially heated to 300° F.

The sulfurized material is then cooled to a temperature of 220° to 230° F. by circulating the material through cooling coils and back to the kettle. When this temperature is reached, 44 pounds of phosphorous sesqui-sulfide is added slowly over a period of ½ hour of continuous agitation. The steam is again turned on at such times as is necessary to maintain the temperature at 220° to 230° F. After the addition of phosphorus, agitation is continued for a period of approximately five hours while the temperature is maintained at 220° to 230° F. At the end of this period the contents of the kettle are immediately cooled to 130° F. by circulation through the exteriorly located cooling coils and pumped to storage.

The phosphorized lubricant may be made as follows: No. 1 lard oil is heated with 10% of phosphorous oxychloride at 170° F. to 200° F. for fifteen minutes. During this time only a slight darkening of the oil occurs. The temperature is slowly increased to 275° F. in order to drive off any remaining phosphorous oxychloride. A black sludge forms in the amount of approximately 25%. 5% of the oil, after it had been decanted from the sludge, was blended with 95% of lubricating oil. This oil had the following characteristics:

|                              |         |
|------------------------------|---------|
| Gravity A. P. I.             | 21-23   |
| Flash °F                     | 530-540 |
| Fire °F                      | 600-610 |
| Viscosity Saybolt at 210° F. | 155-165 |
| Pour °F                      | 20-25   |

Halogenated hydrocarbons have been added to mineral oil in the past to impart E. P. properties. In general, however, they have not been considered satisfactory due to lack of stability as shown particularly by the tendency to hydrolyze. Stable halogenated hydrocarbons are not very effective unless used in large quantities. It has been found, however, that highly halogenated open chain hydrocarbons containing a minimum of approximately 85% chlorine and boiling at approximately 180° C. or above do not substantially hydrolyze at this temperature, when used in small amounts in conjunction with phosphorized or sulfurized and phosphorized oils and they impart unusual E. P. characteristics to these oils. Those halogenated open chain hydrocarbons containing at least two carbon atoms and which have all or all but one of the hydrogen replaced by chlorine, have been found to be quite stable and are very effective E. P. agents when used with phosphorized or phosphorized and sulfurized lubricants. Tetrachlorbutane, for example, though of sufficiently high boiling point (approximately 190° C.) to be satisfactory as an E. P. lubricant is not sufficiently stable. Cold alcoholic potash will immediately decompose tetrachlorbutane, whereas there is no evidence of a reaction with hexachlorethane under similar conditions. Both of these compounds were boiled in water for six hours and the water tested for evidence of hydrolysis of the compounds. It was found that tetrachlorbutane had hydrolyzed to the extent of 1.14%, while hexachlorethane showed negligible hydrolysis, the figure

obtained being 0.07%. Halogenated hydrocarbons which have been found suitable as extreme pressure agents according to this invention are highly halogenated aliphatic compounds which do not boil under about 180° C. and which do not substantially hydrolyze at this temperature. Examples of such compounds are hexachlorethane, heptachlorpropane, octachlorbutane, and numerous others. The matter of boiling point is important from the standpoint of the practical application of the lubricant. Lower boiling compounds may be volatilized and lost at the temperatures encountered in actual service.

The halogenated compounds may be lubricants themselves or may be used in connection with mineral lubricating oils which already contain an extreme pressure base as a phosphorized or a sulfurized and phosphorized oil base or in connection with the phosphorized or sulfurized and phosphorized base alone which may be a lubricant in itself. The stable halogenated compounds when blended in small quantities in mineral lubricating oil do not produce high Timken or S. A. E. tests. However, when they are added in small quantities to sulfurized-phosphorized lubricants which already possess the ability to withstand high loads on the Timken machine, the S. A. E. test of the blend is increased out of all proportion from what would be expected on a basis of tests of the stable halogenated compounds in mineral oil. As examples of lubricants within the scope of this invention and in order to provide a comparison with existing lubricants, the following table has been compiled. All of the lubricants tested were of approximately the same viscosity and were within the viscosity range of S. A. E. 90.

Table I

|    | Material                               | Timken test         |                      | S. A. E.<br>test, load<br>at 1000<br>R. P. M. |
|----|----------------------------------------|---------------------|----------------------|-----------------------------------------------|
|    |                                        | Beam<br>arm<br>load | Pressure             |                                               |
| 45 | Mineral oil                            | Pounds 12           | Pounds/sq. in. 7,000 | Pounds 15-50                                  |
|    | 82% mineral oil                        | 86                  | 36,500               | 90                                            |
| 50 | 18% sulfurized and phosphorized base   | 68                  | 13,000               | 90                                            |
|    | 94% mineral oil                        | 59                  | 15,000               | 90                                            |
|    | 6% hexachlorethane                     | 77                  | 18,000               | 400                                           |
|    | 96% mineral oil                        | 77                  | 19,500               | 530                                           |
|    | 4% hexachlorethane                     | 77                  | 33,750               | 380                                           |
| 55 | 10% hexachlorethane                    | 86                  | 36,500               | 340                                           |
|    | 80% mineral oil                        | 86                  | 33,750               | 520                                           |
|    | 20% hexachlorethane                    | 77                  | 34,500               | 550                                           |
|    | 78.7% mineral oil                      | 86                  | 36,500               | 340                                           |
|    | 17.3% sulfurized and phosphorized base | 86                  | 33,750               | 380                                           |
| 60 | 4.0% hexachlorethane                   | 86                  | 36,500               | 340                                           |
|    | 78.7% mineral oil                      | 86                  | 33,750               | 520                                           |
|    | 17.3% sulfurized and phosphorized base | 86                  | 36,500               | 340                                           |
|    | 4.0% heptachlorpropane                 | 86                  | 36,500               | 340                                           |
| 65 | 79.6% mineral oil                      | 86                  | 36,500               | 340                                           |
|    | 17.5% sulfurized and phosphorized base | 86                  | 36,500               | 340                                           |
|    | 3.0% hexachlorethane                   | 86                  | 36,500               | 340                                           |
|    | 77.3% mineral oil                      | 86                  | 36,500               | 340                                           |
|    | 17.1% sulfurized and phosphorized base | 86                  | 36,500               | 340                                           |
|    | 5.0% hexachlorethane                   | 86                  | 36,500               | 340                                           |
| 70 | 78% mineral oil                        | 86                  | 36,500               | 340                                           |
|    | 22% sulfurized and phosphorized base   | 86                  | 36,500               | 340                                           |
|    | 95% mineral oil                        | 68                  | 17,000               | 320                                           |
|    | 5% chlorinated n-heptane <sup>1</sup>  | 86                  | 17,550               | 335                                           |

<sup>1</sup> Chlorinated to 64% chlorine by weight.

<sup>2</sup> Chlorinated to 63% chlorine by weight.

It will be noted from the above results that mineral oil alone, as might be expected, shows very low results on both the Timken and S. A. E.

machines. When 18% of a sulfurized and phosphorized base is added to the mineral oil, the Timken test is greatly increased, while the S. A. E. test is increased only a small amount. The addition of 4% or 6% of hexachlorethane to mineral oil increases the pressure as measured by the Timken machine, and as measured by the S. A. E. machine only a relatively small amount. It will be noted that although the Timken beam arm load is appreciably increased, the pressure per square inch remains fairly low as calculated from the width of the scar formed on the test block at the point of frictional contact between the test block and cup. With a given beam arm load, the calculated pressure varies inversely with the width of the scar. However, when 3-5% of hexachlorethane is added to a mineral oil which already contains 18% of a sulfurized and phosphorized base, the Timken test remains high, while the S. A. E. test increases vastly over what would be anticipated based on the tests in straight mineral oil. The fact that in some cases there was a small decrease in the Timken test when the chlorine compound was added to the sulfurized-phosphorized lubricant is not considered significant since the amount of the decrease is within the accuracy of the machine. That this unusual increase is not simply due to the increase in the total amount of E. P. agents present is evident by the sum of the results on the blend of mineral oil containing 22% of a sulfurized and phosphorized base and on the blend of mineral oil and 4% or 6% hexachlorethane which is considerably less than the S. A. E. test of 340-520 lbs. shown by the preferred blends.

During the course of this investigation it was noted that several chlorinated aliphatic compounds were unusual in their behavior in that they showed a high S. A. E. test when blended with straight mineral oil. Reference to Table I shows that 5% of chlorinated n-heptane (64% Cl content) or 5% of chlorinated iso-octane (63% Cl content) when blended with 95% straight mineral oil produced an unusually high S. A. E. test for this class of compounds. Fur-

play, as in turning a corner. The thrust machine alternately loads and unloads these washers four times a minute. The load is adjusted at the start of the test and may be varied from 1000 to 5000 lbs. per square inch. The amount of wear on the bronze washer is inversely related to the lubricating quality of the lubricant under test. The results of these tests are given in Table II.

10

Table II

|    |                                        | Hours run<br>at 5000 lbs.<br>per sq. in. | Loss of<br>washer metal<br>in grams |
|----|----------------------------------------|------------------------------------------|-------------------------------------|
| 15 | Mineral oil, S. A. E. 00               | 12                                       | 1.028                               |
|    | 82% mineral oil                        | 2                                        | 0.507                               |
|    | 18% sulfurized and phosphorized base   |                                          |                                     |
|    | 96% mineral oil                        | 2                                        | 0.410                               |
|    | 4% hexachlorethane                     |                                          |                                     |
|    | 79.5% mineral                          |                                          |                                     |
|    | 17.5% sulfurized and phosphorized base | 2                                        | 0.095                               |
| 20 | 3.0% hexachlorethane                   |                                          |                                     |
|    | 86.4% mineral oil                      |                                          |                                     |
|    | 9.6% sulfurized and phosphorized base  | 2                                        | 0.030                               |
|    | 4.0% hexachlorethane                   |                                          |                                     |

<sup>1</sup> 3000 lbs./sq. in. load. (Would not hold greater load.)

25

It is apparent from the data in Table II that the combinations of mineral oil, sulfurized and phosphorized base and hexachlorethane give considerably better results, indicating less wear and superior lubricating properties, than would be expected from the tests on either the sulfurized and phosphorized base or hexachlorethane when blended with mineral oil. In addition to the wear being less with the preferred combination of materials, the appearance of the bronze washers after being tested with the preferred lubricants is far superior to that obtained with the other lubricants. There is much less scratching and marking of the metal surface of the washer.

30

35

40

Further tests were made by putting a preferred form of the lubricant into the differentials of a number of new motor cars all of which had hypoid gears. Table III gives the composition of the lubricants used and the results obtained.

45

Table III

| Car                 | Mineral oil      | Sulfurized and phosphorized base | Hexachloroethane | Mileage | Backlash | Timken test |              | S. A. E. load at 1,000 R. P. M. |
|---------------------|------------------|----------------------------------|------------------|---------|----------|-------------|--------------|---------------------------------|
|                     |                  |                                  |                  |         |          | Beam load   | Pressure     |                                 |
| '38 Plymouth        | Per cent<br>78.7 | Per cent<br>17.3                 | Per cent<br>4.0  |         | Inches   |             | Lbs./sq. in. |                                 |
|                     |                  |                                  |                  | 0       | 0.006    |             |              |                                 |
|                     |                  |                                  |                  | 4,100   | 0.006    |             |              |                                 |
|                     |                  |                                  |                  | 11,500  | 0.006    |             |              |                                 |
|                     |                  |                                  |                  | 0       | 0.006    |             |              |                                 |
|                     |                  |                                  |                  | 2,670   | 0.006    |             |              |                                 |
|                     |                  |                                  |                  | 0       | 0.006    |             |              |                                 |
|                     |                  |                                  |                  | 5,270   | 0.0065   |             |              |                                 |
|                     |                  |                                  |                  | 0       | 0.006    |             |              |                                 |
|                     |                  |                                  |                  | 9,949   | 0.006    |             |              |                                 |
| '38 Chevrolet       | 78.5             | 17.5                             | 3.0              |         |          |             |              |                                 |
| '38 Chrysler Royale | 79.5             | 17.5                             | 3.0              |         |          |             |              |                                 |

ther investigation showed that these compounds were unstable and for this reason they are unsatisfactory as E. P. additives even though a high S. A. E. test was obtained. This lack of stability in these compounds accounts for the high S. A. E. tests since in general a more chemically active chlorine would be expected to show higher E. P. characteristics.

Tests of these lubricants have also been made in a device known as a "thrust machine" designed to simulate the action of the bronze spacer washers in the differential assembly of a rear axle. These washers are located in back of the differential or "spider" gears and receive sudden and severe loads whenever the gears come into

65 The maximum wear on any of the indicated sets of gears is shown by the increase in backlash of 0.0065" obtained on the Chevrolet. In addition the gears were not scuffed, scratched or discolored, thereby further showing the unusual properties of this lubricant.

Not only do my lubricants have high E. P. properties and reduce wear as shown in the foregoing tables of data, but the corrosion on ferrous metals ordinarily encountered with various chlorinated compounds used in mineral lubricating oil as E. P. additives, is substantially, if not entirely eliminated. Comparative tests on samples of ferrous metals were made by partially immersing small samples of the metals in min-

eral oil containing 6% of hexachlorethane at a temperature of approximately 460° F. Similar samples were tested in an identical manner using the same mineral oils, blended with 6% hexachlorethane and 18% of a sulfurized and phosphorized base. In the former tests the metal pieces were discolored by the presence of a dark brown layer of material, indicating that the surface of the metal had been attacked. In the tests where the sulfurized and phosphorized base formed part of the blend, the metal surfaces after the test remained clean and bright and showed no evidence of any corrosion. It is apparent from these results that the sulfurized and phosphorized base has an inhibiting action on the corrosive properties at elevated temperatures of hexachlorethane in mineral oil. The metal samples used were small sections of ferrous sheet stock known as "shim stock" and the journals normally used in the Faville-Levalley lubricant testing machine.

It is recognized that the temperature selected for the test is well above the temperature usually approached by a body of lubricant even under conditions of high rubbing loads, but it is also well established that the metal surfaces at the points of frictional contact achieve temperatures well above the temperature of the indicated corrosion tests. For this reason the corrosion test results presented are believed to give a good indication of the behavior to be anticipated by E. P. lubricants under actual service conditions.

It is obvious the quantity of halogenated compound used may vary within rather wide limits although from approximately 1% to 6% is generally preferred where E. P. characteristics are important. The upper limit of 6% has been mentioned only because with the methods of testing now available it has been found that maximum results can be obtained by adding this amount. There does not appear to be any reason, however, why quantities in excess of 6% may not be used. The quantity of phosphorized or sulfurized and phosphorized base preferably varies from approximately 5% to 25%, although these proportions are not critical and the invention contemplates the use of these materials in proportions outside the preferable limits.

While the foregoing data and discussion relate to the addition of stable halogenated aliphatic hydrocarbons to mineral oil containing a sulfurized and phosphorized E. P. base, it is within the scope of this invention to add halogenated hydrocarbon directly to a phosphorized or a sulfurized and phosphorized E. P. base and to use this base as a lubricant or to add it to mineral oil and use the resulting mixture as a lubricant, or to bring about any mixture of the aforementioned components in any one of a number of ways that will be obvious to those skilled in the art.

It has also been found that these lubricants containing a phosphorized or sulfurized and phosphorized base and a stable halogenated hydrocarbon are excellent cutting fluids for machine cutting tools as well as grinding and drawing oils. They may be used either straight or emulsified with water. The most noticeable characteristics of the performance of these lubricants as cutting fluids are the increased life of the cutting edge of the tool used and the improved bright, clean-looking finish on the machined surface.

What I claim is:

1. A lubricant comprising mineral lubricating oil, a phosphorized fatty oil and a stable highly halogenated aliphatic hydrocarbon having a boiling point not substantially below 180° C.
2. A lubricant comprising mineral lubricating oil, a phosphorized and sulfurized fatty oil and a stable highly halogenated aliphatic hydrocarbon having a boiling point not substantially below 180° C.
3. A lubricant comprising a phosphorized fatty oil and a stable highly halogenated aliphatic hydrocarbon having a boiling point not substantially below 180° C.
4. A lubricant comprising a phosphorized and sulfurized fatty oil and a stable highly halogenated aliphatic hydrocarbon having a boiling point not substantially below 180° C.
5. A lubricant comprising mineral lubricating oil, a phosphorized fatty oil and a stable highly chlorinated aliphatic hydrocarbon having a boiling point not substantially below 180° C.
6. A lubricant comprising mineral lubricating oil, a phosphorized and sulfurized fatty oil and a stable highly chlorinated aliphatic hydrocarbon having a boiling point not substantially below 180° C.
7. A lubricant comprising a phosphorized fatty oil and a stable highly chlorinated aliphatic hydrocarbon having a boiling point not substantially below 180° C.
8. A lubricant comprising a phosphorized fatty oil and a stable highly chlorinated aliphatic hydrocarbon having a boiling point not substantially below 180° C. and containing not less than 85% chlorine.
9. A lubricant comprising a phosphorized and sulfurized fatty oil and a stable highly chlorinated aliphatic hydrocarbon having a boiling point not substantially below 180° C.
10. A lubricant comprising a phosphorized and sulfurized fatty oil and a stable highly chlorinated aliphatic hydrocarbon having a boiling point not substantially below 180° C. and containing not less than 85% chlorine.
11. A lubricant comprising mineral lubricating oil, a phosphorized fatty oil and a stable highly halogenated aliphatic hydrocarbon having a boiling point not substantially below 180° C. and in which all of the hydrogen has been replaced by halogen.
12. A lubricant comprising mineral lubricating oil, a phosphorized fatty oil and a stable highly chlorinated aliphatic hydrocarbon having a boiling point not substantially below 180° C. and in which all of the hydrogen has been replaced by chlorine.
13. A lubricant comprising mineral lubricating oil, sulfurized and phosphorized fatty oil and hexachlorethane.
14. A lubricant comprising mineral lubricating oil, sulfurized and phosphorized fatty oil and heptachlorpropane.
15. A lubricant comprising approximately 1% to 6% hexachlorethane, 5% to 25% sulfurized and phosphorized fatty oil, and mineral oil.
16. A lubricant comprising approximately 1% to 6% heptachlorpropane, 5% to 25% sulfurized and phosphorized fatty oil, and mineral oil.
17. A lubricant comprising a major portion of mineral lubricating oil, a minor proportion of phosphorized fatty oil and halogenated aliphatic hydrocarbon boiling not substantially below 180° C.

18. A lubricant in accordance with claim 17 where the halogen is chlorine.
19. A lubricant comprising mineral lubricating oil, phosphorized fatty oil and a stable highly halogenated aliphatic hydrocarbon having a boiling point not substantially below 180° C., which hydrocarbon is selected from the group consisting of two to four carbon atom hydrocarbons.
20. A lubricant comprising mineral lubricating oil, phosphorized and sulfurized fatty oil and a stable highly halogenated aliphatic hydrocarbon having a boiling point not substantially below 180° C., which hydrocarbon is selected from the group consisting of two to four carbon atom hydrocarbons.
21. A lubricant comprising mineral lubricating oil, sulfurized and phosphorized fatty oil and octachlorbutane.
22. A lubricant comprising mineral lubricating oil, phosphorized fatty oil and octachlorbutane.
23. Method of lubricating relatively moving metallic surfaces in frictional engagement with each other which comprises bringing in contact and chemically reacting therewith at the point of frictional engagement a lubricant composition comprising mineral lubricating oil, phosphorized fatty oil and a stable highly halogenated aliphatic hydrocarbon having a boiling point not substantially below 180° C.
24. Method of lubricating relatively moving metallic surfaces in frictional engagement with each other which comprises bringing in contact and chemically reacting therewith at the point of frictional engagement a lubricant composition comprising phosphorized and sulfurized fatty oil and stable highly halogenated aliphatic hydrocarbon having a boiling point not substantially below 180° C.
25. Method of lubricating relatively moving metallic surfaces in frictional engagement with each other which comprises bringing in contact and chemically reacting therewith at the point of frictional engagement a lubricant composition comprising approximately 1% to 6% hexachlorethane, 5% to 25% sulfurized and phosphorized fatty oil and mineral oil.
26. Method of lubricating relatively moving metallic surfaces in frictional engagement with each other which comprises bringing in contact and chemically reacting therewith at the point of frictional engagement a lubricant composition comprising approximately 1% to 6% heptachloropropane, 5% to 25% sulfurized and phosphorized fatty oil and mineral oil.

WILLIAM A. WHITTIER.